

[54] FUEL AND LUBRICATING OIL ADDITIVES  
TRANSITION METAL COMPLEXES

[75] Inventors: William T. Brannen, West Lake,  
Ohio; Roger W. Watson, Highland,  
Ill.

[73] Assignee: Standard Oil Company, Chicago, Ill.

[22] Filed: Oct. 10, 1969

[21] Appl. No.: 865,496

[52] U.S. Cl. .... 44/68, 252/33

[51] Int. Cl. .... C10I 1/24

[58] Field of Search .... 252/18, 33, 32.5, 34; 44/68,  
44/DIG. 2

[56] References Cited

UNITED STATES PATENTS

|           |         |               |          |
|-----------|---------|---------------|----------|
| 3,535,241 | 10/1970 | Revukas.....  | 252/32.5 |
| 2,851,417 | 9/1958  | Andress ..... | 252/25   |
| R26,433   | 8/1968  | Le Suer ..... | 252/34   |

|           |         |                     |        |
|-----------|---------|---------------------|--------|
| 2,464,497 | 3/1949  | Giammaria .....     | 252/34 |
| 3,306,908 | 2/1967  | Le Suer .....       | 252/35 |
| 3,351,647 | 11/1967 | Butler et al. ....  | 252/34 |
| 2,294,525 | 9/1942  | Waugh.....          | 252/34 |
| 2,976,238 | 3/1961  | Elliott et al. .... | 252/33 |
| 3,649,661 | 3/1972  | Otto et al. ....    | 252/33 |

Primary Examiner—Patrick P. Garvin

Assistant Examiner—L. Vaughn

Attorney, Agent, or Firm—Arthur G. Gilkes; William T. McClain

[57] ABSTRACT

The disclosure describes the reaction product produced by the reaction of about equal molar portions of (1) an alkyl benzene sulfonic acid, an alkyl sulfonic acid, an alkyl phosphorus acid or an alkyl carboxylic acid having an average molecular weight between about 200 and about 1600 and (2) a transition metal complexed with a polyamine.

1 Claim, No Drawings

## FUEL AND LUBRICATING OIL ADDITIVES TRANSITION METAL COMPLEXES

### BACKGROUND OF THE INVENTION

In many cases it is desirable to have an additive for hydrocarbon fuels which conducts static electricity from the fuel to ground. Such a fuel additive is termed an antistatic agent. These agents are commonly employed by hydrocarbon fuel manufacturers to prevent static charge build up in fuels while they are in transit and thereby reduce the possibility of explosions. The main considerations in formulating an antistatic agent are finding the minimum concentration, the least expensive components and the most inert formula possible. The purpose of such considerations is to minimize possible undesirable effects of the antistatic agent and produce a low cost antistatic agent.

Alternatively, it is desirable in formulating antistatic agents to find one which is multifunctional. That is, it is desirable to have an antistatic agent which may inhibit oxidation, enhance lubricating properties of the fuel or lubricant to which it is added and/or suspend foreign material to prevent accumulation and deposits on metal surfaces. Frequently, it is the case that multifunctional agents have been discovered but have been too expensive to incorporate as antistatic agents. Also many times such antistatic agents tend to deposit in the induction system of the engine and build up to effect engine performance (the term "induction system" as used herein is intended to mean the path that the incoming air follows in an automobile engine through the air cleaner, carburetor and intake manifold into the cylinders. This air is of course an air-gasoline mixture after passing through the carburetor.) The problem is then to find an inexpensive antistatic agent that will be multifunctional and will not itself deposit further along the induction system of the engine.

Another important property of antistatic agents is inertness to other additives which may be incorporated into the hydrocarbon fuel or lubricating oil. Reaction would of course deplete the effective additive in the fuel or lubricating oil and tend to reduce its overall efficiency as well as increase the need for additional additive. Most desirable, then, is an antistatic agent which readily disperses into the hydrocarbon fuel or lubricating oil and serves as a conductive agent, yet remains inert to other active additives in such fuel or lubricating oil.

### SUMMARY OF THE INVENTION

Briefly, the invention can be described as the reaction product produced by the reaction between about equal molar portions of (1) an alkyl benzene sulfonic acid, an alkyl sulfonic acid, an alkyl phosphoric acid or an alkyl carboxylic acid having an average molecular weight between about 200 and about 1,600, and (2) a transition metal complex of a polyamine.

The reaction product is proposed as a hydrocarbon

fuel or lubricating oil additive. It would be used in hydrocarbon fuels in a concentration of from about 0.0001 percent to about 0.5 percent based upon the weight of hydrocarbon fuel. As a fuel additive, the reaction product acts as an antistatic agent, reducing the build up of static electricity during the loading or unloading of fuel. In lubricating oils the reaction product can be added in amounts ranging from about 0.1 percent to about 10 percent based on the weight of oil of lubricating viscosity. As a lubricating oil additive, the reaction product acts as an antistatic agent and inhibits oxidation and wear of metal surfaces as well.

Transition metal complexes useful in the invention of this disclosure are described in The Journal of the American Chemical Society in volume 88 at pages 2156 through 2162 (1966), hereby incorporated by reference. Nonlimiting examples of metal salts useful in forming transition metal complexes are the transition metal chlorides, perchlorates, nitrates, thiocyanates, oxalates, bromides and fluoborates. Nonlimiting examples of the transition metals are those selected from the group consisting of cadmium, chromium, cobalt, copper, iron, manganese, molybdenum, mercury, nickel, rhodium, silver, titanium, tungsten and zinc.

Any polyamine can be complexed with the various transition metals. Suitable polyamines generally come within the formula  $H_2N(-alkylene-NH)_nH$ , in which n is an integer from about 1 to about 12, and 'alkylene' is a saturated divalent hydrocarbon containing from about 1 to about 10 carbon atoms. Suitable polyamines include, for example, butylene polyamines, and cyclic homologues of such polyamines, for example, piperazines. Specific examples of alkylene polyamines are: ethylene diamine, hexamethylene diamine, diethylene triamine, triethylene tetramine, tetraethylene pentamine, hexaethyleneheptamine and N-2-aminoethyl-piperazine. Polyethylene polyamines are generally preferred, pentaethylenehexamine being particularly preferred since the transition metals generally form hexacoordinate complexes.

### PREFERRED EMBODIMENTS

For simplicity in the following examples, the designations below shall mean an alkyl substituent attached to an alkyl benzene sulfonic acid, alkyl sulfonic acid, alkyl phosphorus acid or alkyl carboxylic acid having an average molecular weight and an average number of carbon atoms as follows:

| Designation | Average Molecular Weight | Average Number of Carbon Atoms |
|-------------|--------------------------|--------------------------------|
| L-4         | 280                      | 20                             |
| L-10        | 320                      | 23                             |
| L-50        | 420                      | 30                             |
| H-100       | 920                      | 66                             |

### EXAMPLE I

An alkyl benzene sulfonic acid, alkyl sulfonic acid, alkyl phosphorus acid or alkyl carboxylic acid can be reacted at a temperature in the range of about 100°F. to about 350°F. for about one-half to about ten hours in approximately equal molar quantities with a transition metal complex. Such a complex can be prepared by reacting equimolar amounts of  $CrCl_3$  with pentaethylenehexamine (PEHA) in methanol at a temperature in the range of from about 70°F. to about 300°F. for about one-half to about ten hours, or prepared as

exemplified in The Journal of the American Chemical Society (previously cited).

The alkyl benzene sulfonic acid is preferably one wherein the alkyl substituent is a branched chain hydrocarbon having an average molecular weight in the range of from about 50 to about 1,450, thereby giving the acid an average molecular weight of from about 200 to about 1,600. Specific examples of such acids are L-4 benzene sulfonic acid, L-10 benzene sulfonic acid, L-50 benzene sulfonic acid and H-100 benzene sulfonic acid.

The alkyl sulfonic acid is preferably one wherein the alkyl substituent is a branched chain hydrocarbon having an average molecular weight in the range of from about 100 to about 1,500, thereby giving the acid an average molecular weight of from about 200 to about 1,600. Specific examples of such acids are L-4 sulfonic acid, L-10 sulfonic acid, L-50 sulfonic acid and H-100 sulfonic acid.

The alkyl phosphorus acid is preferably one wherein the alkyl substituent is a branched chain hydrocarbon having an average molecular weight in the range of from about 100 to about 1,500, thereby giving the acid an average molecular weight of from about 200 to

about 1600. Specific examples of such acids are L-4 phosphorus acid, L-10 phosphorus acid, L-50 phosphorus acid and H-100 phosphorus acid.

The alkyl carboxylic acid is preferably one wherein the alkyl substituent is a branched chain hydrocarbon having an average molecular weight in the range of from about 150 to about 1550, thereby giving the acid an average molecular weight of from about 200 to about 1,600. Specific examples of such acids are L-4 carboxylic acid, L-10 carboxylic acid, L-50 carboxylic acid, H-100 carboxylic acid, oleic acid, linoleic acid, eluidic acid and eleostearic acid.

What is claimed is:

1. Gasoline containing 0.0001 to 0.5 weight percent of a metal complex consisting essentially of the reaction product of equimolar amounts of (a) an alkylbenzene sulfonic acid having an average molecular weight of from about 200 to about 1,600 and containing only alkyl substituents, and (b) the equimolar complex of chromium chloride and pentaethylenehexamine, wherein said reaction product being formed at from about 100°F. to about 350°F. and said complex being formed at from about 70°F. to about 300°F.

\* \* \* \* \*

25

30

35

40

45

50

55

60

65